

## UNITED STATES PATENT OFFICE

2,350,688

## METALLIC SOAP COMPOSITION

Francis J. Licata, New York, N. Y., and Joseph Nothum, Elizabeth, N. J., assignors to National Oil Products Company, Harrison, N. J., a corporation of New Jersey

No Drawing. Application August 3, 1940,  
Serial No. 351,110

16 Claims. (Cl. 106—243)

This invention relates to polyvalent metal soaps and to polyvalent metal soap solutions suitable for waterproofing purposes.

As is well known in the art, aluminum soaps such as aluminum stearate, aluminum palmitate and the like may be dissolved in solvents such as toluol, etc. in order to form solutions which are useful for waterproofing materials such as bricks, cloth, paper, etc. While these solutions have many valuable properties and have been widely used, the aluminum soaps contained therein are ordinarily not very soluble in easily available solvents, as is evidenced by the fact that the solutions now on the market usually contain only about 2% to 3% of the soap. Hence storage or transportation of such solvents necessitates storing or transporting large quantities of solvent, which is not particularly economical. Moreover it is usually not feasible to store or ship the aluminum soap and then prepare the desired solution when needed, since these soaps tend to become more and more insoluble with age. As a result there has been an extensive demand in the industry for stable aluminum soap solutions containing substantially more than 2% to 3% of the soap.

It has been proposed to employ aluminum soap solutions for waterproofing textiles and other fibrous materials; this proposal has met with some degree of success because of the excellent waterproofing properties imparted to the textiles by soaps such as aluminum stearate. However, it has been found that soaps of the type of aluminum stearate are relatively soluble in petroleum hydrocarbon solvents and hence tend to be washed from textiles or other materials upon contact with such solvents. Thus, there is a great demand for a polyvalent metal soap which will effectively waterproof fibrous materials and yet resist the action of petroleum hydrocarbon solvents.

It may also be desirable in certain cases to produce polyvalent metal soaps having melting points somewhat higher than those of typical polyvalent metal soaps now on the market. For example, aluminum stearate is often mixed with paraffin wax in order to raise the softening point of the paraffin wax and thus make it more suitable for waterproofing objects to be subjected to somewhat elevated temperatures. While this use of aluminum stearate has met with considerable success, there has been a demand for a soap which could be mixed with paraffin wax so as to yield a mixture having a somewhat higher melt-

ing point than is attainable with aluminum stearate.

It is an object of this invention to provide novel polyvalent metal soaps.

5 It is a more specific object of this invention to provide solutions of polyvalent metal soaps which may be employed for waterproofing purposes so as to yield objects having waterproof coatings resistant to the action of petroleum hydrocarbon solvents.

10 It is a further object of this invention to provide polyvalent metal soap compositions which may be blended with materials such as paraffin wax to yield products having relatively high melting points.

15 We have found that polyvalent metal soaps, the fatty portions of which are derived from hydrogenated castor oil or the corresponding fatty acids, possess properties which make them ex-

20 tremely suitable for a wide variety of purposes. In the first place these soaps have considerably higher melting points than the corresponding soaps derived from other fatty acids; hence they may be blended with paraffin wax in order to give mixtures having softening points much higher than those heretofore attainable. In the second place the polyvalent metal soaps of our invention

25 are soluble in many relatively high boiling lacquer solvents of the polar type but tend to be relatively insoluble in non-polar solvents such as the petroleum hydrocarbons. Because of the solubility of the polyvalent metal soaps of our invention in such lacquer solvents, solutions of

30 polyvalent metal soaps in such solvents are made available to the trade for waterproofing purposes; this factor is advantageous because it permits the production of useful polyvalent metal soap solutions employing solvents which could not heretofore be used for preparing such solutions, and

35 thus the field of usefulness of polyvalent metal soaps is considerably broadened. Moreover the polyvalent metal soaps of our invention are capable of producing waterproof coatings upon fibrous materials which are resistant to petroleum hydrocarbon solvents; hence these fibrous materials may be subjected to drycleaning or

40 other similar operations without losing their waterproof characteristics. Our novel soaps may be easily and economically prepared and because of 45 their many important properties will find great use in the trade.

45 The aluminum soaps of our invention may be prepared by reacting an alkali metal soap prepared from hydrogenated castor oil or the corresponding fatty acids with a suitable aluminum

salt such as aluminum sulfate. The hydrogenated castor oil may be formed by hydrogenating castor oil in any suitable manner and may have an iodine value between about 1 and about 15. The alkali metal soap is most advantageously made by saponifying hydrogenated castor oil or the fatty acids derived therefrom with an alkali such as sodium hydroxide. The reaction of the sodium soap thus formed with the aluminum sulfate is preferably carried out by dissolving the sodium soap in water and then adding sufficient aluminum sulfate to the solution, which is preferably heated, e. g. to about 80° C., so as to cause substantially complete precipitation of the aluminum soap. The aluminum soap thus obtained may then be washed free of soluble salts, dried and ground in the usual manner. Lead, calcium and zinc soaps of hydrogenated castor oil may also be prepared by following the general method outlined above. However other methods for the preparation of our novel soaps may be employed, if desired.

The polyvalent metal soaps of our invention are generally white powders. These soaps usually have higher melting points than those of the corresponding soaps derived from other fatty acids. Thus the aluminum soap of our invention melts at 160° C. and the lead soap between 130° and 136° C.; the corresponding stearates melt at about 140° C. and 105° C. respectively. Analysis indicates that our novel compounds are constituted chiefly of soaps of 12-hydroxy stearic acid. The aluminum soap of our invention is somewhat soluble in toluol but has a higher gel point in this solvent than aluminum stearate. Because of their relatively high melting points, the soaps of our invention are of particular value for blending with paraffin wax in order to substantially increase the softening point of the paraffin wax without detrimentally affecting the waterproofing characteristics thereof. Other uses for these soaps of our invention will be evident to those skilled in the art from the above description of their properties.

Our extensive experimentations with regard to the solubility of the polyvalent metal soaps of our invention have led us to the conclusion that these soaps are generally soluble in relatively high boiling lacquer solvents of the polar type; as is well known, most metallic soaps, e. g. aluminum stearate, are not soluble in such solvents, and hence it has not been possible to employ these readily available solvents for the preparation of polyvalent metal soap solutions. For example, we have found that the aluminum soap of our invention forms stable, clear solutions in solvents such as butanol, amyl acetate, ethylene glycol monoethylether, diethylene glycol monoethylether and the like. The aluminum soap of our invention also possesses the unique property of being soluble in castor oil. Our experiments have also demonstrated that our novel soaps are relatively insoluble in petroleum hydrocarbon solvents such as solvent naphtha and the like.

It is a relatively simple matter to prepare solutions of the polyvalent metal soaps of our invention in relatively high boiling lacquer solvents of the polar type, since it is only necessary to heat a suitable amount of the soap with the solvent until complete solution is effected and then permit the solution to cool. The amount of polyvalent metal soap which may be dissolved in such solvents may vary widely depending upon the particular solvent employed; however stable solutions containing anywhere from about 5% to 75

about 35% of the aluminum soap may easily be prepared. It is to be understood that small amounts of other aluminum soaps may be added to these solutions in order to suitably modify their properties; when incorporating other soaps in the solutions of our invention, it is sometimes advantageous to add small quantities of solvents such as toluol which are capable of readily dissolving the added soaps. Other ingredients such as emulsifiers, stiffeners, plasticizers, fluidifiers, etc. compatible with the solutions may also be incorporated therein.

The solutions of our invention are particularly adaptable for waterproofing fibrous materials of all kinds; thus, for example, textile materials waterproofed with the solutions of our invention not only have highly effective water-resistant coatings deposited thereon, but the coatings retain their water-resistance even after prolonged contact with the petroleum hydrocarbon solvents used for drycleaning purposes. Our waterproofing solutions also will find application for preparing water impervious tubings to be used as conduits for petroleum hydrocarbon solvents such as gasoline, kerosene and the like. The solutions of our invention may also be employed for waterproofing bricks and similar articles and for other uses well known in the art.

The following examples are illustrative of our invention; amounts are given in parts by weight.

#### Example I

1,000 parts of hydrogenated castor oil having an iodine value of about 4.2 were saponified by reaction with an aqueous solution containing 167 parts of caustic soda. The sodium soap thus obtained was then dissolved in water in amounts sufficient to give a soap concentration of about 10%. The temperature of the solution was then raised to about 80° C. and sufficient aluminum sulfate solution was added to completely react with the soap. After the aluminum soap had completely settled from the solution, it was withdrawn, washed, dried and ground to a powder. The resulting product was a white powder having a melting point of about 160° C.; it blended easily with any desirable amounts of paraffin wax.

#### Example II

50 70 parts of butanol were heated to a temperature of about 70° C., and 30 parts of the aluminum soap of hydrogenated castor oil prepared as described in Example I were dissolved therein. Upon cooling, a stable, completely fluid solution was obtained, which was found to be highly suitable for waterproofing purposes.

#### Example III

60 95 parts of amyl acetate were heated to a temperature of about 70° C., and 5 parts of the aluminum soap of hydrogenated castor oil prepared in accordance with Example I were dissolved therein. Upon cooling, a stable, completely fluid solution was obtained, which was found to be highly suitable for waterproofing purposes.

#### Example IV

70 95 parts of ethylene glycol monoethyl ether were heated to about 70° C. and 5 parts of the aluminum soap of hydrogenated castor oil prepared as described in Example I were dissolved therein. Upon cooling, a stable, completely fluid solution was obtained, which was found to be highly suitable for waterproofing purposes.

*Example V*

95 parts of castor oil were heated to a temperature of about 130° C. and 5 parts of the aluminum soap of hydrogenated castor oil prepared as described in Example I were dissolved therein, whereby a slightly thickened solution was obtained. Upon cooling, the solution remained perfectly clear.

*Example VI*

1000 parts of hydrogenated castor oil having an iodine value of about 4 were saponified by reaction with an aqueous solution containing 137 parts of caustic soda. The sodium soap thus obtained was then dissolved in water in amounts sufficient to give a soap concentration of about 10%. The temperature of the solution was then raised to about 63° C. and sufficient lead acetate solution was added to completely react with the soap. After the lead soap had settled from the solution, it was withdrawn, washed, dried and ground to a powder. The resulting product was a white powder having a melting point between 130° and 136° C.

*Example VII*

1000 parts of hydrogenated castor oil having an iodine value of about 4 were saponified by reaction with an aqueous solution containing 170 parts of caustic soda. The sodium soap thus obtained was then dissolved in water in amounts sufficient to give a soap concentration of about 10%. The temperature of the solution was then raised to about 65° C. and sufficient calcium chloride solution was added to completely react with the soap. After the calcium soap had settled from the solution, it was withdrawn, washed, dried and ground to a powder.

From the above description it will be evident that our invention provides new and valuable polyvalent metal soap compositions which may be employed to great advantage for waterproofing articles of all types. The unique resistance of the polyvalent metal soaps of our invention to the solvent action of petroleum hydrocarbon solvents makes these soaps superior to polyvalent metal soaps heretofore employed for waterproofing purposes. Therefore our invention will undoubtedly be of great interest to those engaged in the manufacture of aluminum and other polyvalent metal soaps.

The term "polyvalent metal soap" is used throughout the specification and claims in the usual manner to include higher fatty acid soaps of heavy metals such as aluminum, calcium, zinc and lead.

Since certain changes in carrying out the above process and certain modifications in the compositions which embody the invention may be made without departing from its scope, it is intended that all matter contained in the above description shall be interpreted as illustrative and not in a limiting sense.

Having described our invention, what we claim as new and desire to secure by Letters Patent, is:

1. A composition of matter comprising chiefly a polyvalent metal soap of 12-hydroxy stearic acid.
2. A composition of matter comprising chiefly the aluminum soap of 12-hydroxy stearic acid.
3. A composition of matter comprising chiefly the calcium soap of 12-hydroxy stearic acid.
4. A composition of matter comprising chiefly the lead soap of 12-hydroxy stearic acid.
- 10 5. A composition of matter comprising chiefly a solution of a polyvalent metal soap of 12-hydroxy stearic acid in a relatively high boiling lacquer solvent of the polar type.
6. A composition of matter comprising chiefly 15 a solution of an aluminum soap of 12-hydroxy stearic acid in a relatively high boiling lacquer solvent of the polar type.
7. A composition of matter comprising chiefly 20 a solution of an aluminum soap of 12-hydroxy stearic acid in butanol.
8. A composition of matter comprising chiefly a solution of an aluminum soap of 12-hydroxy stearic acid in amyl acetate.
9. A composition of matter comprising chiefly 25 a solution of an aluminum soap of 12-hydroxy stearic acid in ethylene glycol monoethylether.
10. A process for preparing solutions suitable 30 for waterproofing purposes, which comprises dissolving a polyvalent metal soap of 12-hydroxy stearic acid in a relatively high boiling lacquer solvent of the polar type.
11. A process for preparing solutions suitable 35 for waterproofing purposes, which comprises dissolving the aluminum soap of 12-hydroxy stearic acid in a relatively high boiling lacquer solvent of the polar type.
12. A process for preparing solutions suitable 40 for waterproofing purposes, which comprises dissolving the aluminum soap of 12-hydroxy stearic acid in butanol.
13. A process for preparing solutions suitable 45 for waterproofing purposes, which comprises dissolving the aluminum soap of 12-hydroxy stearic acid in amyl acetate.
14. A process for preparing solutions suitable 50 for waterproofing purposes, which comprises dissolving the aluminum soap of 12-hydroxy stearic acid in ethylene glycol monoethylether.
15. A process for waterproofing fibrous materials 55 which comprises impregnating the fibrous material with a solution of a polyvalent metal soap of 12-hydroxy stearic acid in a relatively high boiling lacquer solvent of the polar type and evaporating the solvent from the impregnated material.
16. A process for waterproofing fibrous materials which comprises impregnating the fibrous material with a solution of the aluminum soap of 12-hydroxy stearic acid in a relatively high boiling lacquer solvent of the polar type and evaporating the solvent from the impregnated material.

FRANCIS J. LICATA.  
JOSEPH NOTHUM.